

June 2, 1936.

F. G. BRIGHT

2,042,826

PROCESS OF TREATING WOOD

Filed May 31, 1934

2 Sheets-Sheet 1



June 2, 1936.

F. G. BRIGHT

2,042,826

PROCESS OF TREATING WOOD

Filed May 31, 1934

2 Sheets-Sheet 2



Inventor

Frank G. Bright

Witness.

Jedney Peeling

By Henry J. Miller  
Attorney

## UNITED STATES PATENT OFFICE

2,042,826

## PROCESS OF TREATING WOOD

Frank G. Bright, St. Jean, Quebec, Canada, assignor to The Singer Manufacturing Company, Elizabeth, N. J., a corporation of New Jersey

Application May 31, 1934, Serial No. 728,382  
In Canada September 8, 1933

5 Claims. (Cl. 21—12)

This invention relates to improvements in the method of treating wood, and has for its primary object to provide a commercially practicable process of coloring lumber as well as relatively thin wood pieces such as veneers and the like, under conditions resulting in the requisite uniformity of coloring of the treated wood throughout its width and thickness.

Another object of this invention is to provide an improved method of reducing the moisture content of wood to a desired percentage of moisture. A further object of the invention is to provide a process of coloring wood by impregnation under conditions controlled to predetermine the desired moisture content of the wood after being colored. Other and more specific objects of the invention will be apparent from the following description and claims.

For the purpose of obtaining a better understanding of the invention, there is somewhat diagrammatically illustrated in the accompanying drawings one embodiment of apparatus particularly adapted for practising the improved wood-coloring process comprising the present invention, it being understood of course that the invention is not limited to the specific details of construction and the arrangement of parts of an apparatus as herein described, and that modifications thereof or other forms of construction may be employed in practising the present improved wood-treating process.

In the drawings, Fig. 1 is a longitudinal vertical section, partly in side elevation, of a preferred embodiment of the apparatus. Fig. 2 is an end elevation of the apparatus as viewed from the right in Fig. 1. Fig. 3 diagrammatically illustrates the connections for the heat radiating means within the receptacle. Fig. 4 is a detail view in side elevation of the door clamps and showing the cylinder and door flanges in section.

According to the present improved process, it is not essential that the wood before being treated be either initially partially or wholly dried, as a separate operation, although it is desirable that all the wood treated in one run has approximately the same percentage of moisture to insure the same degree of coloring throughout.

The wood to be treated is piled or stacked upon a truck or other suitable carrier, with superposed layers or pieces of the wood separated by suitable spacing strips. The truck or carrier supporting the wood is placed in a suitable receptacle which is then closed preparatory to treating the wood. As illustrated in the accompanying drawings, a preferred embodiment of the receptacle referred

to comprises a substantially horizontally disposed cylindrical body 1 having at its opposite ends removable doors 2.

The doors 2 are each secured in receptacle-closing position by a plurality of releasable clamps comprising bolts 3 extending through notches or slots 4 provided in juxtaposed peripheral end-flanges 5 and 6 of the body 1 and the respective doors. The bolts 3 for each door are hinged upon an endless cable 7 embracing the body 1 adjacent to the end flanges 5 thereof, said bolts being secured in door clamping position by suitable nuts 8. Preferably a suitable gasket 9 is disposed between the flanges 5 and 6 to tightly seal the end openings of the cylindrical body 1. By partly unthreading the nuts 8, the bolts 3 may each be swung outwardly about the cable 7, thereby withdrawing the bolts from the flange notches 4 and releasing the doors 2. When released from their clamping bolts, the doors 2 are each supported by cables 11 connected to a trolley 12 riding a guide-rail 13 extending cross-wise of the cylinder 1, the guide-rails 13 being so disposed with respect to the ends of the cylinder 1 that there is a gravitational tendency for the doors 2 to swing slightly away from the ends of the cylinder 1, so that said doors may be readily shifted by movement of the trolleys 12 to completely expose the ends of the cylinder. Draw-bridge rails 14 pivotally connect floor rails 15 with rails 16 provided within the cylinder 1 for a truck 17 upon which the wood W (Fig. 2) to be treated is piled.

After the wood to be treated has been placed in the receptacle and the doors 2 have been tightly closed, a forced circulation of the atmosphere within the receptacle is induced by starting the operation of fans preferably disposed interiorly of the receptacle and herein later described. At the same time steam is admitted to heat radiators, also later described, it being understood that when treating wood in successive runs the receptacle temperature may be approximately 200° F. before said steam admission, due to the heated condition of the receptacle in the previous treatment and the temperature drop incidental to opening the receptacle doors for removal and insertion of wood.

At about the same time that steam is admitted into the radiators and the operation of the fans started, a vacuum of approximately 26" is created in the receptacle by any suitable means such as an air-pump, ejector or siphon evacuator, the air within the receptacle and a considerable quantity of the air in the wood interstices

being withdrawn therefrom through a pipe 18 and a pipe 19 connected therewith, thus effecting by the reduction of external pressure a lowering of the boiling point of any moisture in the wood, 5 and of course also reducing the temperature limit at which rapid evaporation of said moisture begins. While it is preferred, in order to expedite the process, to start the operation of the fans and to admit steam into the heat radiators 10 before the vacuum step, it is obvious that the order of procedure up to this point may be wholly or in part reversed.

The time required to draw the requisite vacuum is very short, and, dependent upon the character 15 of the air-exhausting apparatus employed need take only a few minutes. Furthermore, the specified vacuum need not be held for any considerable period of time, but immediately after it is attained a definite quantity of ammonia gas may be introduced into the receptacle, which ammonia gas is promptly and thoroughly diffused throughout the receptacle by the fan-induced circulation, whereby all the wood undergoing treatment is acted 20 upon by the ammonia gas from the beginning of 25 the introduction of said gas to insure uniformity of coloring.

Because of the partial vacuum in the receptacle, the initial heated condition thereof, the constant admission of steam into the radiators 30 and the fan-induced circulation past the radiators, the temperature within the receptacle initially rises at a decidedly more rapid rate than the pressure created by introduction of the ammonia gas and the formation of water vapors 35 generated by the heating of the wood. This differential between the relatively low pressure within the receptacle and a pressure normally corresponding to the attained temperature is peculiarly favorable to drying the wood, because 40 the heating of the wood under the low pressure permits an initial vaporization of the surface moisture of the wood and, as the wood becomes gradually heated to a uniform temperature throughout its cellular structure, there results a 45 continuous passage of moisture from the interior of the wood through the outer layers thereof and in a continuous evaporation of said moisture. As the wood is consequently progressively dried from the interior outward, premature hardening is prevented of the outer layers 50 of the wood before the drying action is completed to the desired extent.

The temperature rise should preferably not exceed 350° F., and the above described drying 55 action of the wood during the coloring thereof by impregnation is controlled, as hereinafter described, to meet the conditions incidental to the moisture content of the wood at the beginning of the coloring operation and the desired moisture content at the end of the operation. For 60 this purpose, when the difference between the initial and final moisture content of the wood necessitates a drying action throughout the coloring operation, suitable relief valves provided upon 65 the receptacle containing the wood may be employed to limit the developed pressure below the pressure normally corresponding to the temperature attained at any degree of rise of the latter. The water vapors given off by the wood being constantly circulated past the heated radiators by 70 the fans become superheated and serve as a further wood drying agent, so that while the drying of the wood is progressive it is nevertheless accelerated by the forced circulation. However, 75 it is obvious that the drying action may be ar-

rested during the coloring operation, if desired, by setting the relief valves so that the gases or vapors introduced or liberated within the receptacle may build up a pressure in excess of the pressure corresponding to the attained temperature. 5

A still more positive and more definitely controllable method of arresting the drying of the wood at any time during the coloring operation consists in introducing into the receptacle a pressure building medium such as compressed air, to superimpose a pressure upon the wood additional to that raised by water vapor and gas, whereby at any point in the coloring operation the pressure may be caused to exceed that normally corresponding to the temperature of steam in the receptacle, thus arresting further evaporation of moisture from the wood during continuance of the coloring operation. When the wood to be colored initially has a moisture content which is 20 substantially equal to the desired moisture content after the coloring operation has been completed, the compressed air may be introduced into the receptacle immediately after introduction of the aqua ammonia or ammonia gas, i. e., before the 25 wood has become sufficiently heated to discharge some of its moisture by vaporization, thereby preventing any wood drying action. The pressure developed, or incurred, holds a portion of the wood acids in the wood cells, which acids in 30 conjunction with the heat and ammonia gas effect coloring of the wood. The compressed air may be introduced into the receptacle through the air-pump connection pipe 18, or by means of any other suitable connection between an 35 air-supply line and the receptacle.

The heating of the wood in itself serves to change the color thereof, but instead of employing the deleterious high temperature and length of treatment that would otherwise be necessary 40 by heat treatment alone to obtain darker shades of coloring, the heat coloring action is supplemented by ammonia gas. As the ammonia gas is introduced into the receptacle while the latter is under the vacuum drawn, as before noted, but 45 primarily because of the highly turbulent gaseous condition induced throughout the interior of the receptacle by the fans, the ammonia gas is brought forcibly into contact with all of the wood within the receptacle, for the same length of 50 time and to the same degree, thereby insuring a uniformity of absorption by the wood of the gas and a uniform coloring action thereupon by the reaction of the gas with the wood constituents. The time required for the coloring operation 55 depends upon the depth of color desired and also upon the nature of the wood, although the maximum required time is short as compared with the operation time of previously known wood coloring processes. 60

For temperature-raising purposes, the receptacle is preferably provided with four heat-radiators extending substantially the entire length interiorly of the receptacle and arranged perpendicularly to each other to together define a 65 rectangular space for the wood-supporting truck 17. As illustrated in the drawings, each of the radiators comprises two rows of substantially parallel pipes 20 connected at their opposite ends by headers 21 and supported by a suitable framework 22. By referring more particularly to Fig. 3 of the drawings, it will be understood that superheated steam may be supplied through the inlet pipe 23 to a pipe 24 connected to the several radiators which are in turn connected to an 70 75 80 85 90 95

outlet pipe 25 by means of the pipe 26. The receptacle may be additionally provided with a perforated pipe 28 extending lengthwise along the bottom of the receptacle and suitably connected to a steam supply line 29, whereby in special cases steam may be directly introduced into the receptacle.

For inducing the highly turbulent gaseous condition throughout the interior of the receptacle, 10 fans 30, 31, 32, and 33 are installed within the receptacle and preferably, although not necessarily, behind the opposed vertically disposed radiators 20, 21, said fans being disposed in staggered relationship alternately at opposite sides of 15 the receptacle. The fan shafts are journaled in the wall of the receptacle and in suitable outer bearings 34, said fan shafts carrying pulleys 35 of which the two pulleys at one side of the receptacle are connected by a belt 36, and the two 20 pulleys at the opposite side of the receptacle are connected by a belt 37. One of the pulleys 35 is also connected by a belt 40 to a pulley 41 upon one end of a countershaft 42 journaled in suitable bearings at the under side of the receptacle, 25 said countershaft being driven by any suitable means and carrying at its opposite end a pulley 43 connected by a crossed belt 44 to a pulley 35 at the side of the receptacle opposite to that of the pulley connected to the belt 40.

30 The ammonia gas may be supplied by injecting aqua ammonia directly into the bottom of the receptacle, for instance through a pipe connection 50, or said aqua ammonia may be injected into pans suitably disposed within the receptacle. The heated condition of the receptacle effects evaporation of the aqua ammonia and thereby liberation of the ammonia gas. The quantity of aqua ammonia injected into the receptacle is measured to generate approximately 35 from 25 to 29 lbs. of ammonia gas per 1,000 board feet of wood within the receptacle.

If preferred, the specified quantity of ammonia gas may be supplied from an evaporator external to the receptacle and in which the gas is generated, as for instance by heating aqua ammonia. 45 To this end, the apparatus may include an evaporator comprising a cylindrical body 45, disposed below the receptacle 1 and interiorly provided with pipe coils 46 having a steam inlet line 47 and an outlet line 48. The aqua ammonia is admitted into the cylinder 45 through an inlet line 49 and the liberated ammonia gas is directed into the receptacle 1 by the pipe 50. By 50 employment of the external evaporator expedient, the ammonia gas is preheated before admission into the receptacle 1, thereby minimizing refrigeration action by the expansion of the gas when introduced into the receptacle. Obviously, however, the evaporation of aqua ammonia directly within the receptacle also has the advantage of a minimum refrigeration action.

A further substitute for the described methods of introducing ammonia gas into the receptacle 1 consists of employment of anhydrous ammonia 55 containers which may be suitably connected to the receptacle, the gas thus introduced becoming heated by the heated condition of the receptacle.

After the coloring operation has been completed, 60 the pressure may be relieved to atmos-

pheric pressure, the fans may be stopped, and both doors of the receptacle then opened, whereupon the truck containing the colored wood may be withdrawn from one end of the receptacle and directly followed by another truck load of wood 5 entering the receptacle at its other end, thereby not only expediting loading of the receptacle but also minimizing loss of receptacle heat. It may be mentioned that by introducing the ammonia gas in a definite quantity, which has been determined by experiment to be adequate for obtaining the desired shade of coloring of the wood, any ammonia gas which may be left in the receptacle after relieving the pressure therein is so negligible that it may be disregarded and the 10 doors may be promptly opened after the treatment.

Having thus set forth the nature of the invention, what I claim herein is:—

1. The process of treating wood, consisting in 20 subjecting the wood in a closed receptacle to ammonia gas and to heat above the vaporization point of the moisture content of the wood, and governing the moisture content of the wood by introducing into the receptacle a pressure building 25 medium sufficient to prevent evaporation of the moisture content of the wood at a predetermined stage in the coloring operation.

2. The process of treating wood, consisting in 30 subjecting the wood in a closed receptacle to ammonia gas, raising the temperature in the receptacle above 200° F., inducing by fan action a forced circulation of the atmosphere within the receptacle, and governing the moisture content of the wood by introducing into the receptacle 35 a pressure building medium sufficient to prevent evaporation of the moisture content of the wood at a predetermined stage in the coloring operation.

3. The process of treating wood, consisting in 40 subjecting the wood in a closed receptacle to ammonia gas, raising the temperature within the receptacle above 212° F. under a pressure in said receptacle lower than a pressure corresponding to the temperature attained, inducing a forced 45 circulation of the atmosphere within the receptacle by fan action, and maintaining the heated condition of the receptacle and said forced circulation for a definite period.

4. The process of treating wood, consisting in 50 exhausting the air from a closed receptacle containing the wood, subjecting the wood to ammonia gas, raising the temperature within the receptacle above 212° F., inducing a forced circulation of the atmosphere within the receptacle, 55 and maintaining for a definite period a pressure within the receptacle lower than a pressure corresponding to the temperature attained.

5. The process of coloring wood to a predetermined shade, consisting in subjecting wood in a 60 closed receptacle to a measured quantity of ammonia gas and to a predetermined temperature above the vaporization point of the moisture content of the wood, and bringing the ammonia 65 gas forcibly into contact with the wood by inducing and maintaining for a definite period a highly turbulent gaseous condition throughout the interior of the receptacle.